

# United States Patent [19]

Bresson et al.

[11] Patent Number: 4,990,656

[45] Date of Patent: Feb. 5, 1991

[54] POLYAMINE SUBSTITUTED  
DITHIOCARBAMATE AND PROCESS FOR  
PRODUCING THE SAME

[75] Inventors: Clarence R. Bresson, Bartlesville,  
Okla.; Harold W. Mark,  
Summerville, N.C.

[73] Assignee: Phillips Petroleum Company,  
Bartlesville, Okla.

[21] Appl. No.: 470,773

[22] Filed: Jan. 26, 1990

4,462,898 7/1984 Parlman et al. .... 209/166  
4,514,293 4/1985 Bresson et al. .... 209/167  
4,554,068 11/1985 Kimble et al. .... 209/167  
4,554,108 11/1985 Kimble et al. .... 260/455  
4,595,538 6/1986 Kimble et al. .... 260/502.56  
4,601,818 7/1986 Bresson et al. .... 209/166  
4,622,131 11/1986 Bresson et al. .... 209/167  
4,702,821 10/1987 Bresson et al. .... 209/166

## FOREIGN PATENT DOCUMENTS

496683 10/1953 Canada .  
771181 11/1967 Canada ..... 260/455  
771182 11/1967 Canada ..... 260/455  
116045 7/1982 Japan .

## OTHER PUBLICATIONS

Chemical Abstract No. 78: P124002g (1973).

Chemical Abstract No. 80: P70299e (1974).

Primary Examiner—Nicky Chan  
Attorney, Agent, or Firm—Laney, Dougherty, Hessian &  
Beavers

## [57] ABSTRACT

A polyamine substituted dithiocarbamate compound is provided. Also provided are minerals depressant compounds for recovering mineral values from an ore or concentrate wherein the values are recovered in a froth from an aqueous slurry. A process of forming the minerals depressant compounds and an improved ore flotation process using the minerals depressant compounds are also provided.

10 Claims, No Drawings

## [56] References Cited

### U.S. PATENT DOCUMENTS

|           |         |                      |         |
|-----------|---------|----------------------|---------|
| 2,621,143 | 12/1952 | Goodhue et al.       | 167/22  |
| 2,693,485 | 11/1954 | Gobell               | 260/500 |
| 2,862,850 | 12/1958 | Goodhue              | 167/46  |
| 3,194,825 | 7/1965  | Brotherton et al.    | 260/454 |
| 3,248,400 | 4/1966  | Flieg et al.         | 260/313 |
| 3,425,550 | 2/1969  | Baarson et al.       | 209/166 |
| 3,464,551 | 9/1969  | Falvey               | 209/166 |
| 3,484,488 | 12/1969 | Lichtenwalter et al. | 260/585 |
| 3,940,488 | 2/1976  | Frohberger et al.    | 424/286 |

**POLYAMINE SUBSTITUTED  
DITHIOCARBAMATE AND PROCESS FOR  
PRODUCING THE SAME**

This is a continuation of co-pending application Ser. No. 07/214,948 filed on July 5, 1988, abandoned which is a division of Ser. No. 07/115,392, filed Nov. 2, 1987, now U.S. Pat. No. 4,806,234.

**BACKGROUND OF THE INVENTION**

1. Field of the Invention

In one aspect, the present invention relates to minerals depressant compositions useful in an ore flotation process. In other aspects, the present invention relates to a process of forming the minerals depressant compositions and to an improved ore flotation process using the minerals depressant compositions.

2. Description of the Prior Art

Ore flotation whereby mineral values are recovered in a froth from an aqueous slurry containing the ore or a concentrate of the ore is well-known. In the process, the ore is crushed and an aqueous slurry is formed therefrom. Mineral flotation agents known in the art as "collectors" and mineral flotation depressing agents known in the art as "depressants" are added to the slurry along with other additives such as frothing agents and stabilizers.

Collectors are added to the ore slurry to cause desired minerals contained therein to adhere to bubbles of a froth formed on the surface of the slurry so that they are recovered when the froth is skimmed or otherwise removed from the slurry. Typical mineral flotation collectors include xanthates, amines, alkyl sulfates, arene sulfonates, dithiocarbamates, dithiophosphates, thiols, and fuel oils.

In order to increase the mineral selectivity of ore flotation processes, depressants have been developed and used. That is, the depressants are used to reduce the flotation of undesired metals or ores thereby increasing the production of desired metals or ores.

By the present invention a novel compound is provided. It has been found that the compound is useful as a minerals depressant in an ore flotation process. A process of forming the novel compounds and other compounds useful as minerals depressants and a process of using the compounds are also provided.

**SUMMARY OF THE INVENTION**

In one aspect of the present invention there is provided a polyamine substituted dithiocarbamate. It has been found that this compound is useful as a minerals depressant in an ore flotation process. The polyamine substituted dithiocarbamate can be represented by the formula:



wherein  $\text{R}_1$  and  $\text{R}_2$  of the amine substituent are each selected from the group consisting of an aminohydrocarbyl group and a polyaminohydrocarbyl group,  $\text{R}_3$  of the amine substituent is selected from the group consisting of a hydrocarbyl group, an aminohydrocarbyl group and a polyaminohydrocarbyl group,  $\text{M}$  is se-

lected from the group consisting of an alkali metal and an alkaline earth metal and  $x$  is 1 or 2.

In another aspect of the invention, a process for producing compounds useful as minerals depressants, including the polyamine substituted dithiocarbamate, is provided. In the process, carbon disulfide is reacted with a polyamine in an aqueous solution comprising a compound selected from the group consisting of an alkali metal hydroxide and an alkaline earth metal hydroxide, the polyamine being represented by the formula:



wherein  $\text{R}_1$  and  $\text{R}_2$  are each selected from the group consisting of an aminohydrocarbyl group and a polyaminohydrocarbyl group and  $\text{R}_3$  is selected from the group consisting of a hydrocarbyl group, an aminohydrocarbyl group and a polyaminohydrocarbyl group.

In yet another aspect of the present invention, an improved process for the recovery of molybdenum values from an ore containing the same wherein the values are recovered in a froth from an aqueous slurry containing the ore or a concentrate of the ore is provided. In the process, a minerals depressant comprising a compound produced by reacting carbon disulfide with a polyamine in an aqueous alkali metal hydroxide solution or an aqueous alkaline earth metal hydroxide solution is employed. The minerals depressant compound can comprise the polyamine substituted dithiocarbamate.

It is therefore an object of the present invention to provide a polyamine substituted dithiocarbamate compound.

It is also an object of the present invention to provide a process for producing the polyamine substituted dithiocarbamate and other compounds useful as minerals depressants in an ore flotation process.

Another object of the present invention is to provide an improved ore flotation process using the polyamine substituted dithiocarbamate and other compounds produced by reacting carbon disulfide with a polyamine in an aqueous alkali metal hydroxide or alkaline earth metal hydroxide solution as minerals depressants.

Other objects, features and advantages of the invention will be readily apparent to those skilled in the art upon a reading of the description of preferred embodiments which follows.

**DESCRIPTION OF THE PREFERRED  
EMBODIMENTS**

55 In accordance with the present invention, a new and useful compound is provided. It has been found, that the compound is useful as a minerals depressant in an ore flotation process. The compound is a polyamine substituted dithiocarbamate represented by the following formula:



wherein  $\text{R}_1$  and  $\text{R}_2$  of the amine substituent are each selected from the group consisting of an aminohydro-

carbyl group and a polyaminohydrocarbyl group,  $R_3$  of the amine substituent is selected from the group consisting of a hydrocarbyl group, an aminohydrocarbyl group and a polyaminohydrocarbyl group,  $M$  is selected from the group consisting of an alkali metal and an alkaline earth metal and  $x$  is 1 or 2.

M is preferably sodium or potassium. If  $R_1$  and  $R_2$  is an aminohydrocarbyl group, or if  $R_3$  is a hydrocarbyl group, the group preferably contains from about 3 to about 10 carbon atoms. If  $R_1$  or  $R_2$  is a polyaminohydrocarbyl group, the group preferably contains from about 2 to about 4 nitrogen atoms and from about 3 to about 10 carbon atoms. If  $R_3$  is an aminohydrocarbyl group or a polyaminohydrocarbyl group, the group preferably contains from about 1 to about 3 nitrogen atoms and from about 3 to about 10 carbon atoms.

In the most preferred form of the compound as represented by the above formula,  $R_1$  and  $R_2$  are each aminoethyl groups,  $R_3$  is an ethyl group and  $M$  is sodium, i.e., sodium tris(2-aminoethyl)amine monodithiocarbamate.

The minerals depressant compounds of this invention can be produced by reacting carbon disulfide with a polyamine in an aqueous alkali metal hydroxide solution or an aqueous alkaline earth metal hydroxide solution. For example, the polyamine substituted dithiocarbonate of the present invention can be produced as follows:



wherein  $R_1$  and  $R_2$  are each selected from an amino hydrocarbyl group and a polyamino hydrocarbyl group,  $R_3$  is selected from a hydrocarbyl group, an amino hydrocarbyl group and a polyamino hydrocarbyl group,  $M$  is an alkali metal or an alkaline earth metal and  $x$  is 1 or 2.

The resulting aqueous solution containing the depressant compound is the preferred form of use of the depressant compound. Generally, the aqueous solution contains in the range of from about 20 to about 50 parts by weight of the depressant compound per 100 parts by weight of aqueous solution.

If  $R_1$  or  $R_2$  is an aminohydrocarbyl group, or if  $R_3$  is a hydrocarbyl group, the group preferably contains from about 3 to about 10 carbon atoms. If  $R_1$  or  $R_2$  is a polyaminohydrocarbyl group, the group preferably contains from about 2 to about 4 nitrogen atoms and from about 3 to about 10 carbon atoms. If  $R_3$  is an aminohydrocarbyl group or a polyaminohydrocarbyl group, the group preferably contains from about 1 to about 3 nitrogen atoms and from about 3 to about 10 carbon atoms.

The most preferred depressant composition of the invention is formed using a polyamine wherein each of  $R_1$  and  $R_2$  is an aminoethyl group and  $R_3$  is an ethyl group. An aqueous alkali metal hydroxide solution is

preferably used. The alkali metal hydroxide used can be sodium hydroxide or potassium hydroxide, most preferably sodium hydroxide.

In another aspect of the present invention, compounds produced by reacting carbon disulfide with a polyamine in an aqueous alkali metal hydroxide or alkaline earth metal hydroxide solution, including the above-described polyamine substituted dithiocarbamate, are employed as depressants for the recovery of mineral values from an ore or minerals concentrate containing such values. The depressant compounds and compositions of the present invention have special applicability in a froth flotation process wherein molybdenum mineral values are recovered, i.e., the molybdenum is recovered in the froth from an aqueous slurry containing molybdenum ore or a concentrate from the ore. Examples of suitable molybdenum-bearing ores which can be usefully processed in accordance with this invention are molybdenite, wulfenite, powellite and ferromolybdate. Such ores generally contain copper, lead and iron in addition to molybdenum.

In carrying out the flotation process, the slurry generally contains from about 5 to about 75 weight percent solids of one or more of the above-described molybdenum ores or concentrates formed from the ores. Usually the slurry contains in the range of from about 3 to about 70 weight percent solids, the depressants of this invention and one or more mineral collectors, frothing agents and stabilizers. Examples of mineral collectors useful for recovering molybdenum are fuel oils and mineral oils. Frothing agents which are commonly used in the slurry include polypropylene and polyethylene glycols and the corresponding methyl or ethyl ethers. In addition, isophorone and/or methylisobutyl carbinol can be used. Examples of useful stabilizers are pH conditioners such as calcium oxide and polyphosphates.

The amount of the minerals depressant composition utilized, not including water, is generally in the range of from about 0.1 to about 10 pounds of minerals depressant composition per ton of ore or solids in the slurry. Preferably, the quantity of the depressant composition is in the range of from about 0.2 to about 5.0 pounds of depressant per ton of ore, and most preferably in the range of from about 0.5 to about 2 pounds depressant per ton of ore.

A variety of froth flotation apparatus can be used for carrying out this invention. The most commonly used commercial flotation machines are the Agitar (Galigher Company), Denver D-12 (Denver Equipment Company), and the Fagergren (Western Machinery Company).

The following examples further illustrate the invention.

**EXAMPLE 1**

This example describes an ore flotation process test wherein no mineral depressant was used. A charge of 1000 grams of an ore containing copper, lead, iron and molybdenum (Pinto Valley ore), 560 milliliters of tap water, 0.6 grams of lime, 2 drops (0.018 pounds per ton) of an aromatic oil (Orfom MCO), and 1.1 milliliters (0.011 pounds per ton) of a collector (Aerofloat 238) was placed in a ball mill and the mixture was ground for 10 minutes.

The resulting slurry was transferred to a 2.5 liter capacity Denver D-12 flotation cell. An amount of lime sufficient to adjust the pH of the slurry to 8.5 was added

to the cell. Also added to the cell were 1.1 milliliters of sodium isobutyl xanthate, a collector, and 3 drops (0.025 pounds per ton) of a frother (Dowfroth 250). After conditioning the slurry for 1 minute, the slurry was floated for 4 minutes.

Next, the concentrate was transferred to a 1.6 liter capacity Denver D-12 flotation cell. An amount of lime sufficient to adjust the pH of the slurry to 8.5 was added to the cell, and the slurry was conditioned for 2.5 minutes. One drop (0.018 pounds per ton) of an aromatic oil (Orfom MCO) was added to the cell, and the slurry was conditioned for 0.5 minutes and floated for 4 minutes. The final concentrate was then filtered, dried and analyzed.

The procedure was repeated and an average weight percent recovery was calculated from the two runs. The average weight percent recoveries in this example were:

|            |            |
|------------|------------|
| molybdenum | 90%;       |
| copper     | 93.5%;     |
| iron       | 98.4%; and |
| lead       | 56%.       |

Thus, in this test where no minerals depressant was used, the ratio of the average weight percent recoveries for molybdenum and iron (90.0 divided by 89.4) was 1.01.

#### EXAMPLE 2

This example describes the preparation of the minerals depressant compound of this invention.

Sodium hydroxide was dissolved in tap water in a glass, 4-necked, round-bottomed flask fitted with an addition funnel, reflux condenser, and mechanical stirrer. A polyamine [tris(2-aminoethyl)amine] was dissolved in the sodium hydroxide solution. The resulting solution was cooled to about 10° C. with an ice water bath at which time carbon disulfide was added dropwise. As soon as the carbon disulfide addition began, the solution turned yellow/orange, indicating the formation of substituted dithiocarbamate. The reaction flask was maintained at about 10° C. to about 20° C. to prevent the loss of carbon disulfide by evaporation.

The addition of carbon disulfide was completed in about an hour. The reaction mixture was stirred for another hour or until a homogeneous yellow/orange solution indicated that the carbon disulfide had reacted completely. The solution was then allowed to warm to room temperature.

The resulting aqueous solution of tris(2-aminoethyl)amine dithiocarbamate (also called sodium N,N-bis(2-aminoethyl)-2-aminoethyl dithiocarbamate) contained a concentration of the minerals depressant in an amount of about 40 parts by weight per 100 parts by weight of aqueous solution.

#### EXAMPLE 3

This example describes a mineral ore flotation process test similar to that described in Example 1 except for the addition of the minerals depressant compound produced as described in Example 2.

A charge of 1000 grams of the same ore as was utilized in Example 1 (Pinto Valley ore), 560 milliliters of tap water, 0.6 grams of lime, 2 drops (0.018 pounds per ton) of an aromatic oil (Orfom MCO) and 1.1 milliliters (0.011 pounds per ton) of a collector (Aerofloat 23S) was placed in a ball mill and the mixture ground for 10

minutes. The slurry was transferred to a 1.6 liter capacity Denver D-12 flotation cell.

An amount of lime sufficient to adjust the pH of the slurry to 8.5 and 1 drop (0.025 pounds per ton) of a frother (Dowfroth 250) were added to the cell. Also added to the cell were 2 milliliters pounds per ton) of an aqueous solution containing 1 percent by weight of the aqueous solution of minerals depressant composition prepared as described in Example 2.

The slurry was conditioned for 2.5 minutes and 1 drop (0.018 pounds per ton) of an aromatic oil (Orfom MCO) were added to the cell. The slurry was then conditioned for 30 seconds and floated for 4 minutes. After the slurry was floated, the concentrate was filtered, dried and analyzed.

The procedure was repeated and an average weight percent recovery was calculated from the two runs. The average weight percent recoveries in this example were:

|            |            |
|------------|------------|
| molybdenum | 55.6%;     |
| copper     | 17.1%;     |
| iron       | 12.4%; and |
| lead       | 20.4%.     |

Thus, in this test with the minerals depressant of the invention being used, the ratio of the average weight percent recoveries for molybdenum and iron (55.6 divided by 12.4) was 4.48.

From a comparison of the results obtained in Examples 1 and 3, it is evident that the minerals depressant composition of the present invention provided effective depressing of minerals recovery relative to molybdenum recovery.

What is claimed is:

1. A compound represented by the formula



wherein  $R_1$  and  $R_2$  are each an aminohydrocarbyl group,  $R_3$  is a hydrocarbyl group,  $M$  is selected from the group consisting of an alkali metal and an alkaline earth metal, and  $x$  is 1 or 2.

2. The compound of claim 1 wherein  $R_1$  and  $R_2$  are each aminoethyl groups and  $R_3$  is an ethylene group.
3. The compound of claim 1 wherein  $M$  is selected from the group consisting of sodium and potassium.
4. The compound of claim 1 wherein  $R_1$ ,  $R_2$  and  $R_3$  each have from about 3 to about 10 carbon atoms.
5. The compound of claim 1 wherein  $M$  is sodium.
6. The compound of claim 1 wherein  $R_1$  and  $R_2$  are each aminoethyl groups,  $R_3$  is an ethylene group and  $M$  is sodium.
7. The compound of claim 1 wherein said compound is produced by reacting carbon disulfide with a polyamine in an aqueous solution comprising a compound selected from the group consisting of an alkali metal hydroxide and an alkaline earth metal hydroxide, said polyamine being represented by the formula:



wherein  $R_1$  and  $R_2$  are each an aminohydrocarbyl group and  $R_3$  is a hydrocarbyl group.

8. The compound of claim 7 wherein  $R_1$  and  $R_2$  are each aminoethyl groups and  $R_3$  is an ethylene group.

9. The compound of claim 8 wherein said aqueous solution comprises an alkali metal hydroxide selected

from the group consisting of sodium hydroxide and potassium hydroxide.

10. The compound of claim 9 wherein said alkali metal hydroxide is sodium hydroxide.

\* \* \* \* \*

10

15

20

25

30

35

40

45

50

55

60

65

UNITED STATES PATENT AND TRADEMARK OFFICE  
CERTIFICATE OF CORRECTION

PATENT NO. : 4,990,656

DATED : February 5, 1991

INVENTOR(S) : Clarence R. Bresson and Harold W. Mark

It is certified that error appears in the above-identified patent and that said Letters Patent is hereby corrected as shown below:

Column 1, line 46, delete the word "compounds" and substitute the word --compound-- therefor;

Column 3, line 7, delete the word "and" and substitute the word --or-- therefor;

Column 5, line 67, delete "23S" and substitute --238-- therefor; and

Column 6, line 6, insert --(0.8-- between "milliliters" and "pounds".

Signed and Sealed this  
Second Day of June, 1992

Attest:

DOUGLAS B. COMER

Attesting Officer

Acting Commissioner of Patents and Trademarks